



US011242613B2

(12) **United States Patent**  
**Lomasney**

(10) **Patent No.:** **US 11,242,613 B2**  
(b4) **Date of Patent:** **Feb. 8, 2022**

(54) **ELECTRODEPOSITED, NANOLAMINATE COATINGS AND CLADDINGS FOR CORROSION PROTECTION**

(71) Applicant: **MODUMETAL, INC.**, Seattle, WA (US)

(72) Inventor: **Christina A. Lomasney**, Seattle, WA (US)

(73) Assignee: **MODUMETAL, INC.**, Snohomish, WA (US)

(\*) Notice: Subject to any disclaimer, the term of this patent is extended or adjusted under 35 U.S.C. 154(b) by 0 days.

(21) Appl. No.: **16/726,079**

(22) Filed: **Dec. 23, 2019**

(65) **Prior Publication Data**

US 2020/0318245 A1 Oct. 8, 2020

**Related U.S. Application Data**

(60) Division of application No. 14/729,020, filed on Jun. 2, 2015, now Pat. No. 10,544,510, which is a division of application No. 13/314,948, filed on Dec. 8, 2011, now Pat. No. 10,253,419, which is a continuation of application No. PCT/US2010/037856, filed on Jun. 8, 2010.

(60) Provisional application No. 61/185,020, filed on Jun. 8, 2009.

(51) **Int. Cl.**

|                   |           |
|-------------------|-----------|
| <b>C25D 5/14</b>  | (2006.01) |
| <b>C25D 5/18</b>  | (2006.01) |
| <b>C25D 5/00</b>  | (2006.01) |
| <b>C25D 5/10</b>  | (2006.01) |
| <b>C25D 15/00</b> | (2006.01) |
| <b>C23F 17/00</b> | (2006.01) |

(52) **U.S. Cl.**  
CPC ..... **C25D 5/605** (2020.08); **C23F 17/00** (2013.01); **C25D 5/10** (2013.01); **C25D 5/14** (2013.01); **C25D 5/18** (2013.01); **C25D 15/00** (2013.01); **Y10T 428/12493** (2015.01)

(58) **Field of Classification Search**

None  
See application file for complete search history.

(56) **References Cited**

**U.S. PATENT DOCUMENTS**

|             |        |                 |
|-------------|--------|-----------------|
| 2,428,033 A | 9/1947 | Nachtman        |
| 2,436,316 A | 2/1948 | Lum et al.      |
| 2,470,775 A | 5/1949 | Jemstedt et al. |
| 2,558,090 A | 6/1951 | Jemstedt        |

(Continued)

**FOREIGN PATENT DOCUMENTS**

|    |           |         |
|----|-----------|---------|
| CN | 1236024 A | 11/1999 |
| CN | 1380446 A | 11/2002 |

(Continued)

**OTHER PUBLICATIONS**

U.S. Appl. No. 16/582,931, filed Sep. 25, 2019.

(Continued)

*Primary Examiner* — Adam Krupicka

(74) *Attorney, Agent, or Firm* — Seed Intellectual Property Law Group LLP

(57) **ABSTRACT**

Described herein are electrodeposited corrosion-resistant multilayer coating and claddings that comprises multiple nanoscale layers that periodically vary in electrodeposited species or electrodeposited microstructures. The coatings may comprise electrodeposited metals, ceramics, polymers or combinations thereof. Also described herein are methods for preparation of the coatings and claddings.

**17 Claims, 1 Drawing Sheet**



| (56)                  | References Cited |                      |              |         |                       |  |
|-----------------------|------------------|----------------------|--------------|---------|-----------------------|--|
| U.S. PATENT DOCUMENTS |                  |                      |              |         |                       |  |
| 2,642,654 A           | 6/1953           | Ahrens               | 5,326,454 A  | 7/1994  | Engelhaupt            |  |
| 2,678,909 A           | 5/1954           | Jemstedt et al.      | 5,352,266 A  | 10/1994 | Erb et al.            |  |
| 2,694,743 A           | 11/1954          | Ruskin et al.        | 5,378,583 A  | 1/1995  | Guckel et al.         |  |
| 2,706,170 A           | 4/1955           | Marchese             | 5,413,874 A  | 5/1995  | Moysan, III et al.    |  |
| 2,891,309 A           | 6/1959           | Fenster              | 5,431,800 A  | 7/1995  | Kirchhoff et al.      |  |
| 3,090,733 A           | 5/1963           | Brown                | 5,461,769 A  | 10/1995 | McGregor              |  |
| 3,255,781 A           | 6/1966           | Gillespie, Jr.       | 5,472,795 A  | 12/1995 | Atita                 |  |
| 3,282,810 A           | 11/1966          | Odekerken            | 5,489,488 A  | 2/1996  | Asai et al.           |  |
| 3,359,469 A           | 12/1967          | Levy et al.          | 5,500,600 A  | 3/1996  | Moyses                |  |
| 3,362,851 A           | 1/1968           | Dunster              | 5,547,096 A  | 4/1996  | Kleyn                 |  |
| 3,483,113 A           | 12/1969          | Carter               | 5,527,445 A  | 6/1996  | Palumbo               |  |
| 3,549,505 A           | 12/1970          | Hanusa               | 5,545,435 A  | 8/1996  | Steffier              |  |
| 3,616,286 A           | 10/1971          | Aylward et al.       | 5,620,800 A  | 4/1997  | De Leeuw et al.       |  |
| 3,633,520 A           | 1/1972           | Stiglich, Jr.        | 5,660,704 A  | 8/1997  | Murase                |  |
| 3,716,464 A           | 2/1973           | Kovac et al.         | 5,679,232 A  | 10/1997 | Fedor et al.          |  |
| 3,753,664 A           | 8/1973           | Klingemaier et al.   | 5,738,951 A  | 4/1998  | Goujard et al.        |  |
| 3,759,799 A           | 9/1973           | Reinke               | 5,742,471 A  | 4/1998  | Barbee, Jr. et al.    |  |
| 3,787,244 A           | 1/1974           | Schulmeister et al.  | 5,775,402 A  | 7/1998  | Sachs et al.          |  |
| 3,866,289 A           | 2/1975           | Brown et al.         | 5,783,259 A  | 7/1998  | McDonald              |  |
| 3,941,674 A           | 5/1976           | Vanmunster           | 5,798,033 A  | 8/1998  | Uemiya et al.         |  |
| 3,994,694 A           | 11/1976          | Clauss et al.        | 5,800,930 A  | 9/1998  | Chen et al.           |  |
| 3,996,114 A           | 12/1976          | Ehrsam               | 5,828,526 A  | 10/1998 | Kagawa et al.         |  |
| 4,053,371 A           | 10/1977          | Towsley              | 5,912,069 A  | 6/1999  | Yializis et al.       |  |
| 4,105,526 A           | 8/1978           | Lewellen, Jr. et al. | 5,930,085 A  | 7/1999  | Kitade et al.         |  |
| 4,107,003 A           | 8/1978           | Anselrode            | 5,942,096 A  | 8/1999  | Ruzicka et al.        |  |
| 4,191,617 A           | 3/1980           | Hurley et al.        | 5,952,111 A  | 9/1999  | Sugg et al.           |  |
| 4,204,918 A           | 5/1980           | McIntyre et al.      | 5,958,604 A  | 9/1999  | Riabkov et al.        |  |
| 4,216,272 A           | 8/1980           | Clauss               | 6,036,832 A  | 3/2000  | Knol et al.           |  |
| 4,246,057 A           | 1/1981           | Janowski et al.      | 6,036,833 A  | 3/2000  | Tang et al.           |  |
| 4,284,688 A           | 8/1981           | Stücheli et al.      | 6,071,398 A  | 6/2000  | Martin et al.         |  |
| 4,314,893 A           | 2/1982           | Clauss               | 6,143,424 A  | 11/2000 | Jonte et al.          |  |
| 4,405,427 A           | 9/1983           | Byrd                 | 6,143,430 A  | 11/2000 | Miyasaka et al.       |  |
| 4,422,907 A           | 12/1983          | Birkmaier et al.     | 6,193,858 B1 | 2/2001  | Hradil et al.         |  |
| 4,461,680 A           | 7/1984           | Lashmore             | 6,200,452 B1 | 3/2001  | Angelini              |  |
| 4,464,232 A           | 8/1984           | Wakano et al.        | 6,203,936 B1 | 3/2001  | Cisar et al.          |  |
| 4,510,209 A           | 4/1985           | Hada et al.          | 6,212,078 B1 | 4/2001  | Hunt et al.           |  |
| 4,519,878 A           | 5/1985           | Hara et al.          | 6,214,473 B1 | 4/2001  | Hunt et al.           |  |
| 4,540,472 A           | 9/1985           | Johnson et al.       | 6,284,357 B1 | 9/2001  | Lackey et al.         |  |
| 4,543,300 A           | 9/1985           | Hara et al.          | 6,312,579 B1 | 11/2001 | Bank et al.           |  |
| 4,543,803 A           | 10/1985          | Keyasko              | 6,344,123 B1 | 2/2002  | Bhatnagar             |  |
| 4,591,418 A           | 5/1986           | Snyder               | 6,355,153 B1 | 3/2002  | Uzoh et al.           |  |
| 4,592,808 A           | 6/1986           | Doubt                | 6,398,937 B1 | 6/2002  | Menini et al.         |  |
| 4,597,836 A           | 7/1986           | Schaer et al.        | 6,409,907 B1 | 6/2002  | Braun et al.          |  |
| 4,613,388 A           | 9/1986           | Walter et al.        | 6,415,942 B1 | 7/2002  | Fenton et al.         |  |
| 4,620,661 A           | 11/1986          | Slatterly            | 6,461,678 B1 | 10/2002 | Chen et al.           |  |
| 4,652,348 A           | 3/1987           | Yahalom et al.       | 6,466,417 B1 | 10/2002 | Gill                  |  |
| 4,666,567 A           | 5/1987           | Loch                 | 6,468,672 B1 | 10/2002 | Donovan, III et al.   |  |
| 4,670,356 A           | 6/1987           | Sato et al.          | 6,482,298 B1 | 11/2002 | Bhatnagar             |  |
| 4,678,552 A           | 7/1987           | Chen                 | 6,537,683 B1 | 3/2003  | Staschko et al.       |  |
| 4,678,721 A           | 7/1987           | den Broeder et al.   | 6,547,944 B2 | 4/2003  | Schreiber et al.      |  |
| 4,702,802 A           | 10/1987          | Umino et al.         | 6,592,739 B1 | 7/2003  | Sonoda et al.         |  |
| 4,753 H               | 11/1988          | Chen et al.          | 6,725,916 B2 | 4/2004  | Gray et al.           |  |
| 4,795,735 A           | 1/1989           | Uiu et al.           | 6,739,028 B2 | 5/2004  | Sievenpiper et al.    |  |
| 4,834,845 A           | 5/1989           | Muko et al.          | 6,777,831 B2 | 8/2004  | Gutiérrez, Jr. et al. |  |
| 4,839,214 A           | 6/1989           | Oda et al.           | 6,800,121 B2 | 10/2004 | Shahin                |  |
| 4,869,971 A           | 9/1989           | Nee et al.           | 6,884,499 B2 | 4/2005  | Penich et al.         |  |
| 4,885,215 A           | 12/1989          | Yoshioka et al.      | 6,902,827 B2 | 6/2005  | Kelly et al.          |  |
| 4,904,542 A           | 2/1990           | Mroczkowski          | 6,908,667 B2 | 6/2005  | Christ et al.         |  |
| 4,904,543 A           | 2/1990           | Sakakima et al.      | 6,923,898 B2 | 8/2005  | Yoshimura et al.      |  |
| 4,923,574 A           | 5/1990           | Cohen                | 6,979,490 B2 | 12/2005 | Steffier              |  |
| 4,975,337 A           | 12/1990          | Hyner et al.         | 7,581,933 B2 | 9/2009  | Bruce et al.          |  |
| 5,043,230 A           | 8/1991           | Jagannathan et al.   | 7,632,590 B2 | 12/2009 | Punsalan et al.       |  |
| 5,045,356 A           | 9/1991           | Uemura et al.        | 7,736,753 B2 | 6/2010  | Deligianni et al.     |  |
| 5,056,936 A           | 10/1991          | Mahrus et al.        | 8,084,564 B2 | 12/2011 | Kano et al.           |  |
| 5,059,493 A           | 10/1991          | Takahata             | 8,152,985 B2 | 4/2012  | Macary                |  |
| 5,073,237 A           | 12/1991          | Bacher et al.        | 8,177,945 B2 | 5/2012  | Arvin et al.          |  |
| 5,079,039 A           | 1/1992           | Heraud et al.        | 8,192,608 B2 | 6/2012  | Matthews              |  |
| 5,156,729 A           | 10/1992          | Mahrus et al.        | 8,253,035 B2 | 8/2012  | Matsumoto             |  |
| 5,156,899 A           | 10/1992          | Kistrup et al.       | 8,585,875 B2 | 11/2013 | Cummings et al.       |  |
| 5,158,653 A           | 10/1992          | Lashmore et al.      | 8,814,437 B2 | 8/2014  | Braun                 |  |
| 5,190,637 A           | 3/1993           | Guckel               | 8,916,001 B2 | 12/2014 | Pryce Lewis et al.    |  |
| 5,228,967 A           | 7/1993           | Crites et al.        | 9,005,420 B2 | 4/2015  | Tomantschger et al.   |  |
| 5,268,235 A           | 12/1993          | Lashmore et al.      | 9,056,405 B2 | 6/2015  | Sato et al.           |  |
| 5,300,165 A           | 4/1994           | Sugikawa             | 9,080,692 B2 | 7/2015  | Tomomori et al.       |  |
| 5,320,719 A           | 6/1994           | Lasbmore et al.      | 9,115,439 B2 | 8/2015  | Whitaker              |  |
|                       |                  |                      | 9,234,294 B2 | 1/2016  | Whitaker et al.       |  |
|                       |                  |                      | 9,273,932 B2 | 3/2016  | Whitaker et al.       |  |
|                       |                  |                      | 9,732,433 B2 | 8/2017  | Caldwell et al.       |  |

| (56)                  | References Cited               |                          |                                   |         |  |  |
|-----------------------|--------------------------------|--------------------------|-----------------------------------|---------|--|--|
| U.S. PATENT DOCUMENTS |                                |                          |                                   |         |  |  |
| 9,758,891 B2          | 9/2017 Bao                     | 2011/0277313 A1          | 11/2011 Soracco et al.            |         |  |  |
| 9,783,907 B2          | 10/2017 Cai et al.             | 2012/0118745 A1          | 5/2012 Bao                        |         |  |  |
| 9,938,629 B2          | 4/2018 Whitaker et al.         | 2012/0135270 A1          | 5/2012 Wilbuer et al.             |         |  |  |
| 10,041,185 B2         | 8/2018 Sukenari                | 2012/0231574 A1          | 9/2012 Wang                       |         |  |  |
| 10,253,419 B2         | 4/2019 Lomasney                | 2012/0282417 A1          | 11/2012 Garcia et al.             |         |  |  |
| 10,266,957 B2         | 4/2019 Sugawara et al.         | 2013/0052343 A1          | 2/2013 Dieny et al.               |         |  |  |
| 10,472,727 B2         | 11/2019 Lomasney               | 2013/0071755 A1          | 3/2013 Oguro                      |         |  |  |
| 10,513,791 B2         | 12/2019 Lomasney et al.        | 2013/0075264 A1          | 3/2013 Cummings et al.            |         |  |  |
| 10,544,510 B2         | 1/2020 Lomasney                | 2013/0130057 A1          | 5/2013 Caldwell et al.            |         |  |  |
| 10,662,542 B2         | 5/2020 Caldwell et al.         | 2013/0186852 A1          | 7/2013 Dietrich et al.            |         |  |  |
| 10,689,773 B2         | 6/2020 Whitaker et al.         | 2013/0220831 A1          | 8/2013 Vidaurre Heiremans et al.  |         |  |  |
| 10,781,524 B2         | 9/2020 Whitaker et al.         | 2013/0224008 A1          | 8/2013 Cheung et al.              |         |  |  |
| 10,808,322 B2         | 10/2020 Whitaker et al.        | 2013/0323473 A1          | 12/2013 Dietsch et al.            |         |  |  |
| 10,844,504 B2         | 11/2020 Sklar                  | 2014/0163717 A1          | 6/2014 Das et al.                 |         |  |  |
| 10,851,464 B1         | 12/2020 Kobayashi et al.       | 2014/0178637 A1          | 6/2014 Rajagopalan et al.         |         |  |  |
| 10,961,635 B2         | 3/2021 Whitaker                | 2014/0231266 A1          | 8/2014 Sherrer et al.             |         |  |  |
| 11,118,280 B2         | 9/2021 Lomasney et al.         | 2015/0315716 A1          | 11/2015 Whitaker                  |         |  |  |
| 2001/0037944 A1       | 11/2001 Sanada et al.          | 2015/0322588 A1          | 11/2015 Lomasney et al.           |         |  |  |
| 2002/0011419 A1       | 1/2002 Arao et al.             | 2016/0002790 A1          | 1/2016 Whitaker et al.            |         |  |  |
| 2002/0070118 A1       | 6/2002 Schreiber et al.        | 2016/0002803 A1          | 1/2016 Sklar                      |         |  |  |
| 2002/0100858 A1       | 8/2002 Weber                   | 2016/0002806 A1          | 1/2016 Lomasney                   |         |  |  |
| 2002/0179449 A1       | 12/2002 Domeier et al.         | 2016/0002813 A1          | 1/2016 Lomasney                   |         |  |  |
| 2003/0134142 A1       | 7/2003 Ivey et al.             | 2016/0024663 A1          | 1/2016 Lomasney                   |         |  |  |
| 2003/0234181 A1       | 12/2003 Palumbo                | 2016/0047980 A1          | 2/2016 Page et al.                |         |  |  |
| 2003/0236163 A1       | 12/2003 Chaturvedi et al.      | 2016/0145850 A1          | 5/2016 Cook et al.                |         |  |  |
| 2004/0027715 A1       | 2/2004 Hixson-Goldsmith et al. | 2016/0159488 A1          | 6/2016 Roach et al.               |         |  |  |
| 2004/0031691 A1       | 2/2004 Kelly et al.            | 2016/0160863 A1          | 6/2016 Roach et al.               |         |  |  |
| 2004/0067314 A1       | 4/2004 Joshi et al.            | 2016/0214283 A1          | 7/2016 Schick et al.              |         |  |  |
| 2004/0154925 A1       | 8/2004 Podlaha et al.          | 2017/0191177 A1          | 7/2017 Whitaker et al.            |         |  |  |
| 2004/0178076 A1       | 9/2004 Stonas et al.           | 2017/0191179 A1          | 7/2017 Sklar                      |         |  |  |
| 2004/0211672 A1       | 10/2004 Ishigami et al.        | 2017/0275775 A1          | 9/2017 Guadarrama Calderon et al. |         |  |  |
| 2004/0232005 A1       | 11/2004 Hubel                  | 2018/0016694 A1          | 1/2018 Bao                        |         |  |  |
| 2004/0234683 A1       | 11/2004 Tanaka et al.          | 2018/0066375 A1          | 3/2018 Morgan et al.              |         |  |  |
| 2004/0239836 A1       | 12/2004 Chase                  | 2018/0071980 A1          | 3/2018 Lomasney et al.            |         |  |  |
| 2005/0002228 A1       | 1/2005 Dieny et al.            | 2018/0245229 A1          | 8/2018 Whitaker et al.            |         |  |  |
| 2005/0109433 A1       | 5/2005 Danger et al.           | 2019/0309430 A1          | 10/2019 Sklar                     |         |  |  |
| 2005/0205425 A1       | 9/2005 Palumbo et al.          | 2019/0360116 A1          | 11/2019 Collinson et al.          |         |  |  |
| 2005/0221100 A1       | 10/2005 Kirihara et al.        | 2020/0115998 A1          | 4/2020 Lomasney                   |         |  |  |
| 2005/0279640 A1       | 12/2005 Shimoyama et al.       | 2020/0131658 A1          | 4/2020 Lomasney et al.            |         |  |  |
| 2006/0065533 A1       | 3/2006 Inoue et al.            | 2020/0173032 A1          | 6/2020 Lomasney                   |         |  |  |
| 2006/0135281 A1       | 6/2006 Palumbo et al.          | 2020/0277706 A1          | 9/2020 Lomasney et al.            |         |  |  |
| 2006/0135282 A1       | 6/2006 Palumbo et al.          | 2020/0283923 A1          | 9/2020 Lomasney                   |         |  |  |
| 2006/0201817 A1       | 9/2006 Guggemos et al.         | 2020/0318245 A1          | 10/2020 Lomasney                  |         |  |  |
| 2006/0243597 A1       | 11/2006 Matefi-Tempfli et al.  | 2020/0354846 A1          | 11/2020 Whitaker et al.           |         |  |  |
| 2006/0269770 A1       | 11/2006 Cox et al.             | 2020/0392642 A1          | 12/2020 Lomasney                  |         |  |  |
| 2006/0272949 A1       | 12/2006 Detor et al.           | 2021/0054522 A1          | 2/2021 Lomasney et al.            |         |  |  |
| 2006/0286348 A1       | 12/2006 Sauer                  | 2021/0071303 A1          | 3/2021 Whitaker et al.            |         |  |  |
| 2007/0158204 A1       | 7/2007 Taylor et al.           | 2021/0147995 A1          | 5/2021 Sklar                      |         |  |  |
| 2007/0269648 A1       | 11/2007 Schuh et al.           | FOREIGN PATENT DOCUMENTS |                                   |         |  |  |
| 2007/0278105 A1       | 12/2007 Ettel                  | CN                       | 1924110 A                         | 3/2007  |  |  |
| 2008/0063866 A1       | 3/2008 Allen et al.            | CN                       | 101113527 A                       | 1/2008  |  |  |
| 2008/0093221 A1       | 4/2008 Basol                   | CN                       | 101195924 A                       | 6/2008  |  |  |
| 2008/0102360 A1       | 5/2008 Stimits et al.          | DE                       | 102148339 A                       | 8/2011  |  |  |
| 2008/0226976 A1       | 9/2008 Stimits                 | DE                       | 105442011 A                       | 3/2016  |  |  |
| 2008/0245669 A1       | 10/2008 Yoshioka et al.        | DE                       | 39 02 057 A1                      | 7/1990  |  |  |
| 2008/0271995 A1       | 11/2008 Savastiouk et al.      | EP                       | 1 688 518 A2                      | 8/2006  |  |  |
| 2008/0283236 A1       | 11/2008 Akers et al.           | EP                       | 2 189 554 A1                      | 5/2010  |  |  |
| 2009/0004465 A1       | 1/2009 Kano et al.             | JP                       | S47-2005 A                        | 2/1972  |  |  |
| 2009/0101511 A1       | 4/2009 Lochtman et al.         | JP                       | S47-33925 A                       | 11/1972 |  |  |
| 2009/0114530 A1       | 5/2009 Noda et al.             | JP                       | S52-109439 A                      | 9/1977  |  |  |
| 2009/0130424 A1       | 5/2009 Tholen et al.           | JP                       | 58-197292 A                       | 11/1983 |  |  |
| 2009/0130425 A1       | 5/2009 Whitaker                | JP                       | S60-97774 A                       | 5/1985  |  |  |
| 2009/0155617 A1       | 6/2009 Kim et al.              | JP                       | S61-99692 A                       | 5/1986  |  |  |
| 2009/0283410 A1       | 11/2009 Sklar et al.           | JP                       | H01-132793 A                      | 5/1989  |  |  |
| 2010/0078330 A1       | 4/2010 Hyodo                   | JP                       | 2-214618 A                        | 8/1990  |  |  |
| 2010/0116675 A1       | 5/2010 Sklar et al.            | JP                       | H05-251849 A                      | 9/1993  |  |  |
| 2010/0187117 A1       | 7/2010 Lingenfelter et al.     | JP                       | H06-196324 A                      | 7/1994  |  |  |
| 2010/0304063 A1       | 12/2010 McCrea et al.          | JP                       | 07-065347 A                       | 3/1995  |  |  |
| 2010/0304179 A1       | 12/2010 Facchini et al.        | JP                       | H09-119000 A                      | 5/1997  |  |  |
| 2010/0319757 A1       | 12/2010 Oetting                | JP                       | 2000-239888 A                     | 9/2000  |  |  |
| 2011/0111296 A1       | 5/2011 Berdichevsky et al.     | JP                       | 2001-152388 A                     | 6/2001  |  |  |
| 2011/0162970 A1       | 7/2011 Sato                    | JP                       | 2001-181893 A                     | 7/2001  |  |  |
| 2011/0180413 A1       | 7/2011 Whitaker et al.         | JP                       | 2002-53999 A                      | 2/2002  |  |  |
| 2011/0186582 A1       | 8/2011 Whitaker et al.         | JP                       | 2006-035176 A                     | 2/2006  |  |  |
| 2011/0256356 A1       | 10/2011 Tomantschger et al.    | KR                       | 2009-215590 A                     | 9/2009  |  |  |
|                       |                                | KR                       | 2003-0092463 A                    | 12/2003 |  |  |

(56)

## References Cited

## FOREIGN PATENT DOCUMENTS

|    |                 |    |         |
|----|-----------------|----|---------|
| KR | 10-2015-0132043 | A  | 11/2015 |
| SU | 36121           | A1 | 4/1934  |
| WO | 83/02784        |    | 8/1983  |
| WO | 95/14116        |    | 5/1995  |
| WO | 2004/001100     |    | 12/2003 |
| WO | 2007/045466     |    | 4/2007  |
| WO | 2007/138619     |    | 12/2007 |
| WO | 2008/057401     | A2 | 5/2008  |
| WO | 2009/045433     |    | 4/2009  |
| WO | 2011/033775     | A1 | 3/2011  |
| WO | 2011/110346     | A2 | 9/2011  |
| WO | 2012/145750     | A2 | 10/2012 |
| WO | 2013/133762     | A1 | 9/2013  |
| WO | 2017/097300     | A1 | 6/2017  |

## OTHER PUBLICATIONS

- U.S. Appl. No. 16/671,104, filed Oct. 31, 2019.
- “Appendix 1: Literature review (Task 1): Literature review concerning the improvement of galvanneal (GA) coating adherence during shear test of adhesively bonded GA steel sheets,” 70 pages, no date.
- “Low-temperature iron plating,” web blog article found at [http://blog.sina.com.cn/s/blog\\_48ed0a9c0100024z.html](http://blog.sina.com.cn/s/blog_48ed0a9c0100024z.html), published Mar. 22, 2006, 3 pages. (with English translation).
- Adams et al., “Controlling strength and toughness of multilayer films: A new multiscalar approach,” *J. Appl. Phys.* 74(2):1015-1021, 1993.
- Aizenberg et al., “Skeleton of *Euplectella* sp.: Structural Hierarchy from the Nanoscale to the Macroscale,” *Science* 309:215-218, 2005.
- Alfantazi et al., “Synthesis of nanocrystalline Zn—Ni alloy coatings,” *JMSLD5* 15(15):1361-1363, 1996.
- Atanassov et al., “Electrodeposition and properties of nickel-manganese layers,” *Surface and Coatings Technology* 78:144-149, 1996.
- Bakonyi et al., “Electrodeposited multilayer films with giant magnetoresistance (GMR): Progress and problems,” *Progress in Materials Science* 55:107-245, 2010.
- Bartlett et al., “Electrochemical deposition of macroporous platinum, palladium and cobalt films using polystyrene latex sphere templates,” *Chem. Commun.*, pp. 1671-1672, 2000.
- Beattie et al., “Comparison of Electrodeposited Copper-Zinc Alloys Prepared Individually and Combinatorially,” *J. Electrochem. Soc.* 150(11):C802-C806, 2003.
- Bird et al., “Giant Magnetoresistance in Electrodeposited Ni/Cu and Co/Cu Multilayers,” *J. Electrochem. Soc.* 142(4):L65-L66, 1995.
- Blum, “The Structure and Properties of Alternately Electrodeposited Metals,” presented at the Fortieth General Meeting of the American Electrochemical Society, Lake Placid, New York, Oct. 1, 1921, 14 pages.
- Cohen et al., “Electroplating of Cyclic Multilayered Alloy (CMA) Coatings,” *J. Electrochem. Soc.* 130(10):1987-1995, 1983.
- Cowles, “High cycle fatigue in aircraft gas turbines—an industry perspective,” *International Journal of Fracture* 80(2-3):147-163, 1996.
- “Designing with Metals: Dissimilar Metals and The Galvanic Series,” printed Oct. 5, 2017, 3 pages.
- Despic et al., “Electrochemical Formation of Laminar Deposits of Controlled Structure and Composition,” *J. Electrochem. Soc.* 136(6):1651-1657, 1989.
- Dini et al. “On the High Temperature Ductility Properties of Electrodeposited Sulfamate Nickel,” *Plating and Surface Finishing* 65(2):36-40. 1978.
- Eтminanfar et al., “Corrosion resistance of multilayer coatings of nanolayered Cr/Ni electrodeposited from Cr(III)-Ni(II) bath,” *Thin Solid Films* 520:5322-5327, 2012.
- Gasser et al., “Materials Design for Acoustic Liners: an Example of Tailored Multifunctional Materials,” *Advanced Engineering Materials* 6(1-2):97-102, 2004.
- Georgescu et al., “Magnetic Behavior of [Ni/Co—Ni—Mg—N] x n Cylindrical Multilayers prepared by Magnetoelectrolysis,” *Phys. Stat. Sol. (a)* 189(3):1051-1055, 2002.
- Ghanem et al., “A double templated electrodeposition method for the fabrication of arrays of metal nanodots,” *Electrochemistry Communications* 6:447-453, 2004.
- Grimmett et al., “Pulsed Electrodeposition of Iron-Nickel Alloys,” *J. Electrochem. Soc.* 137(11):3414-3418, 1990.
- Hariyanti, “Electroplating of Cu—Sn Alloys and Compositionally Modulated Multilayers of Cu—Sn—Zn—Ni Alloys on Mild Steel Substrate,” Master of Science Thesis, University of Science, Malaysia, Penang, Malaysia, 2007.
- Harris et al., “Improved Single Crystal Superalloys, CMSX-4® (SLS)[La+Y] and CMSX-486®,” *TMS (The Minerals, Metals & Materials Society), Superalloys*, p. 45-52, 2004.
- Huang et al., “Hardness variation and annealing behavior of a Cr—Ni multilayer electroplated in a trivalent chromium-based bath,” *Surface and Coatings Technology* 203:3320-3324, 2009.
- Huang et al., “Characterization of Cr—Ni multilayers electroplated from a chromium(III)-nickel(II) bath using pulse current,” *Scripta Materialia*, 57:61-64, 2007.
- Igawa et al., “Fabrication of SiC fiber reinforced SiC composite by chemical vapor infiltration for excellent mechanical properties,” *Journal of Physics and Chemistry of Solids* 66:551-554, 2005.
- Ivanov et al., “Corrosion resistance of compositionally modulated multilayered Zn—Ni alloys deposited from single bath,” *Journal of Applied Electrochemistry* 33:239-244, 2003.
- Jeong et al., “The Effect of Grain Size on the Wear Properties of Electrodeposited Nanocrystalline Nickel Coatings,” *Scripta Mater.* 44:493-499, 2001.
- Jia et al., “LIGA and Micromolding” Chapter 4, *The MEMS Handbook*, 2nd edition, CRC Press, Boca Raton, Florida, Edited by Mohamed Gad-el-Hak, 2006.
- Kalu et al., “Cyclic voltammetric studies of the effects of time and temperature on the capacitance of electrochemically deposited nickel hydroxide,” *Journal of Power Sources* 92:163-167, 2001.
- Kaneko et al., “Vickers hardness and deformation of Ni/Cu nano-multilayers electrodeposited on copper substrates,” Eleventh International Conference on Intergranular and Interphase Boundaries 2004, *Journal of Material Science* 40:3231-3236, 2005.
- Karimpoor et al., “Tensile Properties of Bulk Nanocrystalline Hexagonal Cobalt Electrodeposits,” *Materials Science Forum* 386-388:415-420, 2002.
- Keckes et al., “Cell-wall recovery after irreversible deformation of wood,” *Nature Materials* 2:810-814, 2003.
- Kirilova et al., “Corrosion behaviour of Zn—Co compositionally modulated multilayers electrodeposited from single and dual baths,” *Journal of Applied Electrochemistry* 29:1133-1137, 1999.
- Kockar et al., “Effect of potentiostatic waveforms on properties of electrodeposited NiFe alloy films,” *Eur. Phys. J. B*(42):497-501, 2004.
- Kruth et al., “Progress in Additive Manufacturing and Rapid Prototyping” *CIRP Annals* 47(2):525-540, 1998.
- Lashmore et al., “Electrodeposited Cu—Ni Textured Superlattices,” *J. Electrochem. Soc.* 135(5):1218-1221, 1988.
- Lashmore et al., “Electrodeposited Multilayer Metallic Coatings,” *Encyclopedia of Materials Science and Engineering*, Supp. vol. 1:136-140, 1988.
- Leisner et al., “Methods for electrodepositing composition-modulated alloys,” *Journal of Materials Processing Technology* 58:39-44, 1996.
- Leith et al., “Characterization of Flow-Induced Compositional Structure in Electrodeposited NiFe Composition-Modulated Alloys” *J. Electrochem. Soc.* 145(8):2821-2833, 1998.
- Lekka et al., “Corrosion and wear resistant electrodeposited composite coatings,” *Electrochimica Acta* 50:4551-4556, 2005.
- Lewis et al., “Stability in thin film multilayers and microlaminates: the role of free energy, structure, and orientation at interfaces and grain boundaries,” *Scripta Materialia* 48:1079-1085, 2003.
- Low et al., “Electrodeposition of composite coatings containing nanoparticles in a metal deposit,” *Surface & Coating Technology* 201:371-383, 2006.

(56)

## References Cited

## OTHER PUBLICATIONS

- Malone, "New Developments in Electroformed Nickel-Based Structural Alloys," *Plating and Surface Finishing* 74(1):50-56, 1987.
- Marchese, "Stress Reduction of Electrodeposited Nickel," *Journal of the Electrochemical Society* 99(2):39-43, 1952.
- Meng et al., "Fractography, elastic modulus, and oxidation resistance of Novel metal-intermetallic Ni/Ni<sub>3</sub>Al multilayer films," *J. Mater. Res.* 17(4):790-796, 2002.
- Naslain et al., "Synthesis of highly tailored ceramic matrix composites by pressure-pulsed CVI," *Solid State Ionics* 141-142:541-548, 2001.
- Naslain, "The design of the fibre-matrix interfacial zone in ceramic matrix composites," *Composites Part A* 29A: 1145-1155, 1998.
- Nicholls, "Advances in Coating Design for High-Performance Gas Turbines," *MRS Bulletin*, p. 659-670, 2003.
- Onoda et al., "Preparation of amorphous/crystalloid soft magnetic multilayer Ni—Co—B alloy films by electrodeposition," *Journal of Magnetism and Magnetic Materials* 126(1-3):595-598, 1993.
- Parkin et al., "Oscillations in Exchange Coupling and Magnetoresistance in Metallic Superlattice Structures: Co/Ru, Co/Cr, and Fe/Cr," *Physical Review Letters* 64(19):2304-2307, 1990.
- Pilone et al., "Model of Multiple Metal Electrodeposition in Porous Electrodes," *Journal of the Electrochemical Society* 153(5):D85-D90, 2006.
- Podlaha et al. "Induced Codeposition: I. An Experimental Investigation of Ni—Mo Alloys," *J. Electrochem. Soc.* 143(3):885-892, 1996.
- Ross, "Electrodeposited Multilayer Thin Films," *Annual Review of Materials Science* 24:159-188, 1994.
- Rousseau et al., "Single-bath Electrodeposition of Chromium-Nickel Compositionally Modulated Multilayers (CMM) From a Trivalent Chromium Bath," *Plating and Surface Finishing*, p. 106-110, 1999.
- Saleh et al., "Effects of electroplating on the mechanical properties of stereolithography and laser sintered parts," *Rapid Prototyping Journal* 10(5):305-315, 2004.
- Sanders et al., "Mechanics of hollow sphere foams," *Materials Science and Engineering* A347:70-85, 2003.
- Sartwell et al., "Replacement of Chromium Electroplating on Gas Turbine Engine Components Using Thermal Spray Coatings," Report No. NRL/MR/6170-05-8890, Naval Research Laboratory, 2005, (207 pages).
- Schwartz, "Multiple-Layer Alloy Plating," ASM Handbook 5: Surface Engineering, p. 274-276, 1994.
- Sherik, "Synthesis, Structure and Properties of Electrodeposited Bulk Nanocrystalline Nickel," Master's Thesis, Queen's University, Ontario, Canada, 1993.
- Shishkovski, "Laser synthesis of functionally graded meso structures and bulk products," FIZMATLIT, Moscow, Russia, pp. 30-38, 2009, (with English Abstract).
- Simunovich et al., "Electrochemically Layered Copper-Nickel Nanocomposites with Enhanced Hardness," *J. Electrochem. Soc.* 141(1):L10-L11, 1994.
- Sperling et al., "Correlation of stress state and nanohardness via heat treatment of nickel-aluminide multilayer thin films," *J. Mater. Res.* 19(11):3374-3381, 2004.
- Srivastava et al., "Corrosion resistance and microstructure of electrodeposited nickel-cobalt alloy coatings," *Surface & Coatings Technology* 201:3051-3060, 2006.
- Stephenson, Jr., "Development and Utilization of a High Strength Alloy for Electroforming," *Plating* 53(2): 183-192, 1966.
- Suresh, "Graded Materials for Resistance to Contact Deformation and Damage," *Science* 292:2447-2451, 2001.
- Switzer et al., "Electrodeposited Ceramic Superlattices," *Science* 247(4941):444-446, 1990.
- Tench et al., "Considerations in Electrodeposition of Compositionally Modulated Alloys," *J. Electrochem. Soc.* 737(10):3061-3066, 1990.
- Tench et al., "Enhanced Tensile Strength for Electrodeposited Nickel-Copper Multilayer Composites," *Metallurgical Transactions A* 15A):2039-2040, 1984.
- Thangaraj et al., "Corrosion behavior of composition modulated multilayer Zn—Co electrodeposits produced using a single-bath technique," *J. of Appl. Electrochem.* 39:339-345, 2009.
- Thangaraj et al., "Surface Modification by Compositionally Modulated Multilayered Zn—Fe Coatings," *Chinese Journal of Chemistry* 26:2285-2291, 2008.
- Tokarz et al., "Preparation, structural and mechanical properties of electrodeposited Co/Cu multilayers," *phys. stat. sol. (c)* 5(11):3526-3529, 2008.
- Touchstone Research Laboratory, Ltd., Material Safety Data Sheet, CFOAM Carbon Foams, 2008. (4 pages).
- Vill et al., "Mechanical Properties of Tough Multiscalar Microlaminates," *Acta metall. mater.* 43(2):427-437, 1995.
- Voevodin et al., "Superhard, functionally gradient, nanolayered and nanocomposite diamond-like carbon coatings for wear protection," *Diamond and Related Materials* 7:463-467, 1998.
- Wearmouth et al., "Electroforming with Heat-Resistant, Sulfur-Harden Nickel," *Plating and Surface Finishing* 66(10):53-57, 1979.
- Weil et al., "Pulsed Electrodeposition of Layered Brass Structures," *Metallurgical Transactions A* 19A:1569-1573, 1988.
- Weil et al., "Properties of Composite Electrodeposits," U.S. Army Research Office, Final Report, Contract No. DAAL03-87-K-0047, 21 pages, 1990.
- Wikipedia, "Gold," URL= <http://en.wikipedia.org/wiki/Gold>, version modified Nov. 3, 12 pages, 2008.
- Wikipedia, "Silver," URL= <http://en.wikipedia.org/wiki/Silver>, version modified Nov. 3, 12 pages, 2008.
- Wilcox, "Surface Modification With Compositionally Modulated Multilayer Coatings," *The Journal of Corrosion Science and Engineering* 6(Paper 52): 2004 (5 pages).
- Wu et al., "Preparation and characterization of superhard CN<sub>x</sub>/ZrN multilayers," *J. Vac. Sci. Technol. A* 15(3):946-950, 1997.
- Yahalom et al., "Formation of composition-modulated alloys by electrodeposition," *Journal of Materials Science* 22:499-503, 1987.
- Yang et al., "Effects of SiC sub-layer on mechanical properties of Tyranno-SA/SiC composites with multiple interlayers," *Ceramics International* 31:525-531, 2005.
- Yang et al., "Enhanced elastic modulus in composition-modulated gold-nickel and copper-palladium foils," *Journal of Applied Physics* 48(3):876-879, 1977.
- Yogesha et al., "Optimization of deposition conditions for development of high corrosion resistant Zn—Fe multilayer coatings," *Journal of Materials Processing Technology* 211:1409-1415, 2011.
- Zabludovsky et al., "The Obtaining of Cobalt Multilayers by Programme-controlled Pulse Current," *Transactions of the Institute of Metal Finishing* 75(5):203-204, 1997.
- U.S. Appl. No. 17/179,351, filed Feb. 18, 2021.
- Paz et al., "Nano-Laminated Alloys for Improved Return on Oilfield Assets," Society of Petroleum Engineers, 2016 (14 pages).
- U.S. Pat. No. 11,118,280, dated Sep. 14, 2021.
- U.S. Appl. No. 17/409,688, dated Aug. 23, 2021.



## 1

## ELECTRODEPOSITED, NANOLAMINATE COATINGS AND CLADDINGS FOR CORROSION PROTECTION

This application is a divisional of U.S. application Ser. No. 14/729,020, filed Jun. 2, 2015, which is a divisional of U.S. application Ser. No. 13/314,948, filed Dec. 8, 2011, now U.S. Pat. No. 10,253,419, issued Apr. 9, 2019, which is a continuation of PCT/US2010/037856, filed Jun. 8, 2010, which claims the benefit of U.S. Provisional Application No. 61/185,020, filed Jun. 8, 2009, each of which is incorporated herein by reference in its entirety.

## BACKGROUND

Laminated metals, and in particular nanolaminated metals, are of interest for structural and thermal applications because of their unique toughness, fatigue resistance and thermal stability. For corrosion protection, however, relatively little success has been reported in the formation of corrosion-resistant coatings that are laminated on the nanoscale.

Electrodeposition has been successfully used to deposit nanolaminated coatings on metal and alloy components for a variety of engineering applications. Electrodeposition is recognized as a low-cost method for forming a dense coating on any conductive substrate. Electrodeposition has been demonstrated as a viable means for producing nanolaminated coatings, in which the individual laminates may vary in the composition of the metal, ceramic or organic-metal composition or other microstructure feature. By time varying electrodeposition parameters such as current density, bath composition, pH, mixing rate, and/or temperature, multi-laminate materials can be produced in a single bath. Alternately by moving a mandrel or substrate from one bath to another, each of which represents a different combination of parameters that are held constant, multi-laminate materials or coatings can be realized.

The corrosion behavior of organic, ceramic, metal and metal-containing coatings depends primarily on their chemistry, microstructure, adhesion, thickness and galvanic interaction with the substrate to which they are applied. In the case of sacrificial metal or metal-containing coatings, such as zinc on an iron-based substrate, the coating is less electronegative than the substrate and so oxidation of the coating occurs preferentially, thus protecting the substrate. Because these coatings protect by providing an oxidation-preferred sacrificial layer, they will continue to work even when marred or scratched. The performance of sacrificial coatings depends heavily on the rate of oxidation of the coating layer and the thickness of the sacrificial layer. Corrosion protection of the substrate only lasts so long as the sacrificial coating is in place and may vary depending on the environment that the coating is subjected to and the resulting rate of coating oxidation.

Alternately, in the case of a barrier coating, such as nickel on an iron-based substrate, the coating is more electronegative than the substrate and thus works by creating a barrier to oxidative corrosion. In A-type metals, such as Fe, Ni, Cr and Zn, it is generally true that the higher the electronegativity, the greater the nobility (non reactivity). When the coating is more noble than the substrate, if that coating is marred or scratched in any way, or if coverage is not complete, these coatings will not work, and may accelerate the progress of substrate corrosion at the substrate: coating interface, resulting in preferential attack of the substrate. This is also true when ceramic coatings are used. For

## 2

example, it has been reported in the prior art that while fully dense TiN coatings are more noble than steel and aluminum in resistance to various corrosive environments, pinholes and micropores that can occur during processing of these coating are detrimental to their corrosion resistance properties. In the case of barrier coatings, pinholes in the coating may accelerate corrosion in the underlying metal by pitting, crevice or galvanic corrosion mechanisms.

Many approaches have been utilized to improve the corrosion resistance of barrier coatings, such as reducing pinhole defects through the use of a metallic intermediate layer or multiple layering schemes. Such approaches are generally targeted at reducing the probability of defects or reducing the susceptibility to failure in the case of a defect, mar or scratch. One example of a multiple layering scheme is the practice commonly found in the deployment of industrial coatings, which involves the use of a primer, containing a sacrificial metal such as zinc, coupled with a highly-crosslinked, low surface energy topcoat (such as a fluorinated or polyurethane topcoat). In such case, the topcoat acts as a barrier to corrosion. In case the integrity of the topcoat is compromised for any reason, the metal contained in the primer acts as a sacrificial media, thus sacrificially protecting the substrate from corrosion.

Dezincification is a term is used to mean the corroding away of one constituent of any alloy leaving the others more or less in situ. This phenomenon is perhaps most common in brasses containing high percentages of zinc, but the same or parallel phenomena are familiar in the corrosion of aluminum bronzes and other alloys of metals of widely different chemical affinities. Dezincification usually becomes evident as an area with well-defined boundaries, and within which the more noble metal becomes concentrated as compared with the original alloy. In the case of brass the zinc is often almost completely removed and copper is present almost in a pure state, but in a very weak mechanical condition. Corrosion by dezincification usually depends on the galvanic differential between the dissimilar metals and the environmental conditions contributing to corrosion. Dezincification of alloys results in overall loss of the structural integrity of the alloy and is considered one of the most aggressive forms of corrosion.

Coatings that may represent the best of both the sacrificial coating and the barrier coating are those that are more noble than the substrate and creates a barrier to corrosion, but, in case that coating is compromised, is also less noble than the substrate and will sacrificially corrode, thus protecting the substrate from direct attack.

## SUMMARY OF THE INVENTION

In one embodiment of the technology described herein, the phenomena observed in dezincification of alloys is leveraged to enable corrosion resistant coatings that are both more and less noble than the substrate, and which protect the substrate by acting both as a barrier and as a sacrificial coating. Other embodiments and advantages of this technology will become apparent upon consideration of the following description.

The technology described herein includes in one embodiment an electrodeposited, corrosion-resistant multilayer coating or cladding, which comprises multiple nanoscale layers that periodically vary in electrodeposited species or electrodeposited microstructures (electrodeposited species microstructures), wherein variations in said layers of said electrodeposited species or electrodeposited species micro-

structure result in galvanic interactions between the layers, said nanoscale layers having interfaces there between.

The technology described herein also provides an electrodeposition method for producing a corrosion resistant multilayer coating or cladding comprising the steps of:

- a) placing a mandrel or a substrate to be coated in a first electrolyte containing one or more metal ions, ceramic particles, polymer particles, or a combination thereof; and
- b) applying electric current and varying in time one or more of: the amplitude of the electrical current, electrolyte temperature, electrolyte additive concentration, or electrolyte agitation, in order to produce periodic layers of electrodeposited species or periodic layer of electrodeposited species microstructures; and
- c) growing a multilayer coating under such conditions until the desired thickness of the multilayer coating is achieved.

Such a method may further comprising after step (c), step (d), which comprises removing the mandrel or the substrate from the bath and rinsing.

The technology described herein further provides an electrodeposition method for producing a corrosion resistant multilayer coating or cladding comprising the steps of:

- a) placing a mandrel or substrate to be coated in a first electrolyte containing one or more metal ions, ceramic particles, polymer particles, or a combination thereof; and
  - b) applying electric current and varying in time one or more of: the electrical current, electrolyte temperature, electrolyte additive concentration, or electrolyte agitation, in order to produce periodic layers of electrodeposited species or periodic layer of electrodeposited species microstructures; and
  - c) growing a nanometer-thickness layer under such conditions; and
  - d) placing said mandrel or substrate to be coated in a second electrolyte containing one or more metal ions that is different from said first electrolyte, said second electrolyte containing metal ions, ceramic particles, polymer particles, or a combination thereof; and
  - e) repeating steps (a) through (d) until the desired thickness of the multilayer coating is achieved;
- wherein steps (a) through (d) are repeated at least two times. Such a method may further comprising after step (e), step (f) which comprises removing the mandrel or the coated substrate from the bath and rinsing.

Also described herein is an electrodeposited, corrosion-resistant multilayer coating or cladding, which comprises multiple nanoscale layers that vary in electrodeposited species microstructure, which layer variations result in galvanic interactions occurring between the layers. Also described is a corrosion-resistant multilayer coating or cladding, which comprises multiple nanoscale layers that vary in electrodeposited species, which layer variations result in galvanic interactions occurring between the layers.

The coating and claddings described herein are resistant to corrosion due to oxidation, reduction, stress, dissolution, dezincification, acid, base, or sulfidation and the like.

#### BRIEF DESCRIPTION OF THE DRAWINGS

FIG. 1 shows a schematic of a substrate having the "Multilayered Coating" of a preferred embodiment (on the left of FIG. 1) and a schematic of a substrate having a "Homogeneous Coating" as is known in the art (on the right of FIG. 1). Both the left and right side schematics represent how a pinhole, a micropore or damage to a coating changes over time (in sequence from the top to the bottom of FIG. 1) relative to the substrate shown on the bottom of each of the sequences. The schematic illustrates a few representative

layers that are not to scale with the substrate. In typical embodiments coating layers are on the nanoscale and present in a greater number than shown in FIG. 1.

#### DETAILED DESCRIPTION

In one embodiment an electrodeposited corrosion-resistant multilayer coating comprised of individual layers with thicknesses on the nanometer scale is provided. In such an embodiment the individual layers can differ in electronegativity from adjacent layers.

In other embodiments, the present technology provides corrosion-resistant multilayer coatings or claddings (together herein referred to as a "coating") that comprise multiple nanoscale layers having variations in the composition of metal, alloy, polymer, or ceramic components, or combination thereof (together herein referred to as "electrodeposited species").

In such embodiments the variations in the compositions between layers results in galvanic interactions occurring between the layers.

In another embodiment, the present technology provides a corrosion-resistant multilayer coating that comprises multiple nanoscale layers having layer variations in grain size, crystal orientation, grain boundary geometry, or combination thereof (together herein referred to as "electrodeposited species microstructure(s)"), which layer variations result in galvanic interactions occurring between the layers.

In another embodiment multilayer coating or cladding is provided for, in which the layers vary in electronegativity or in nobility, and in which the rate of corrosion can be controlled by controlling the difference in electronegativity or in the reactivity (or "nobility") of adjacent layers.

One embodiment of the present technology provides a multilayer coating or cladding in which one of the periodic layers is less noble than the other layer and is less noble than the substrate, thus establishing a periodic sacrificial layer in the multilayer coating.

As used herein "layers that periodically vary" means a series of two or more non-identical layers (non identical "periodic layers") that are repeatedly applied over an underlying surface or mandrel. The series of non-identical layers can include a simple alternating pattern of two or more non-identical layers (e.g., layer 1, layer 2, layer 1, layer 2, etc.) or in another embodiment may include three or more non-identical layers (e.g., layer 1, layer 2, layer 3, layer 1, layer 2, layer 3, etc.). More complex alternating patterns can involve two, three, four, five or more layers arranged in constant or varying sequences (e.g., layer 1, layer 2, layer 3, layer 2, layer 1, layer 2, layer 3, layer 2, layer 1, etc.). In one embodiment, a series of two layers is alternately applied 100 times to provide a total of 200 layers having 100 periodic layers of a first type alternated with 100 periodic layers of a second type, wherein the first and second type of periodic layer are not identical. In other embodiments, "layers that periodically vary" include 2 or more, 3 or more, 4 or more, or 5 or more layers that are repeatedly applied about 5, 10, 20, 50, 100, 200, 250, 500, 750, 1,000, 1,250, 1,500, 1,750, 2,000, 3,000, 4,000, 5,000, 7,500, 10,000, 15,000, 20,000 or more times.

As used herein, a "periodic layer" is an individual layer within "layers that periodically vary".

In another embodiment, the present technology provides a multilayer coating or cladding in which one of the periodic layers is more noble than the other layer and is more noble than the substrate, thus establishing a periodic corrosion barrier layer in the multilayer coating.

In another embodiment, the present technology provides a multilayer coating in which one of the periodic layers is less noble than the adjacent layers and all layers are less noble than the substrate.

In still another embodiment, the present technology provides a multilayer coating or cladding in which one of the periodic layers is more noble than the adjacent layers and all layers are more noble than the substrate.

One embodiment of the present technology provides for a corrosion-resistant multilayer coating or cladding compositions that comprise individual layers, where the layers are not discrete, but rather exhibit diffuse interfaces with adjacent layers. In some embodiments the diffuse region between layers may be 0.5, 0.7, 1, 2, 5, 10, 15, 20, 25, 30, 40, 50, 75, 100, 200, 400, 500, 1,000, 2,000, 4,000, 6,000, 8,000 or 10,000 nanometers. In other embodiments the diffuse region between layers may be 1 to 5, or 5 to 25, or 25 to 100, or 100 to 500, or 500 to 1,000, or 1,000 to 2,000, or 2,000 to 5,000, or 4,000 to 10,000 nanometers. The thickness of the diffuse interface may be controlled in a variety of ways, including the rate at which the electrodeposition conditions are change.

Another embodiment of the technology described herein provides a method for producing a multilayered corrosion-resistant coating that comprises multiple nanoscale layers (“nanolaminates”) that vary in electrodeposited species or electrodeposited species microstructure or a combination thereof, which layers are produced by an electrodeposition process.

Where variations in electrodeposited species or combinations thereof are employed, in some embodiments, the electrodeposited species may comprise one or more of Ni, Zn, Fe, Cu, Au, Ag, Pd, Sn, Mn, Co, Pb, Al, Ti, Mg and Cr, Al<sub>2</sub>O<sub>3</sub>, SiO<sub>2</sub>, TiN, BoN, Fe<sub>2</sub>O<sub>3</sub>, MgO, and TiO<sub>2</sub>, epoxy, polyurethane, polyaniline, polyethylene, poly ether ether ketone, polypropylene.

In other embodiments the electrodeposited species may comprise one or more metals selected from Ni, Zn, Fe, Cu, Au, Ag, Pd, Sn, Mn, Co, Pb, Al, Ti, Mg and Cr. Alternatively, the metals may be selected from: Ni, Zn, Fe, Cu, Sn, Mn, Co, Pb, Al, Ti, Mg and Cr; or from Ni, Zn, Fe, Cu, Sn, Mn, Co, Ti, Mg and Cr; or from Ni, Zn, Fe, Sn, and Cr. The metal may be present in any percentage. In such embodiments the percentage of each metal may independently selected about 0.001, 0.005, 0.01, 0.05, 0.1, 0.5, 1, 5, 10, 15, 20, 25, 30, 30, 35, 40, 45, 50, 55, 60, 65, 70, 75, 80, 85, 90, 95, 98, 99, 99.9, 99.99, 99.999 or 100 percent of the electrodeposited species. Unless otherwise indicated, the percentages provided herein refer to weight percentages.

In other embodiments the electrodeposited species may comprise one or more ceramics (e.g., metals oxides or metal nitrides) selected from Al<sub>2</sub>O<sub>3</sub>, SiO<sub>2</sub>, TiN, BoN, Fe<sub>2</sub>O<sub>3</sub>, MgO, SiC, ZrC, CrC, diamond particulates, and TiO<sub>2</sub>. In such embodiments the percentage of each ceramic may independently selected about 0.001, 0.005, 0.01, 0.05, 0.1, 0.5, 1, 5, 10, 15, 20, 25, 30, 30, 35, 40, 45, 50, 55, 60, 65, 70, 75, 80, 85, 90, 95, 98, 99, 99.9, 99.99, 99.999 or 100 percent of the electrodeposited species.

In still other embodiments the electrodeposited species may comprise one or more polymers selected from epoxy, polyurethane, polyaniline, polyethylene, poly ether ether ketone, polypropylene, and poly(3,4-ethylenedioxythiophene) poly(styrenesulfonate). In such embodiments the percentage of each polymer may independently selected about 0.001, 0.005, 0.01, 0.05, 0.1, 0.5, 1, 5, 10, 15, 20, 25,

30, 30, 35, 40, 45, 50, 55, 60, 65, 70, 75, 80, 85, 90, 95, 98, 99, 99.9, 99.99, 99.999 or 100 percent of the electrodeposited species.

Another embodiment of the present technology provides a electrodeposition method for producing a nanolaminated, corrosion resistant coating which reduces through-hole defects in the overall corrosion resistant coating. Such methods include those wherein multi-layered coatings or claddings are applied to a substrate or mandrel as illustrated in FIG. 1.

As shown on the left of FIG. 1, the multilayer coating of a preferred embodiment is disposed to have two alternating (light and dark) layers covering a substrate. In the embodiment of the left side of FIG. 1, the light layer is a protective layer and the dark layer is a sacrificial layer. As the sequence shows, over time the hole in the light layer expands slightly in a direction parallel to the surface of the substrate, and the sacrificial dark layer under the damaged light layer is consumed in a direction parallel with the surface of the substrate. It is also noted that the hole in the outermost (exposed) layer of the multilayer coating does not expand to breach the second light layer disposed between the hole and the substrate, thereby protecting the substrate from corrosion. In a preferred embodiment, corrosion is confined to the less-noble layers (the dark layers), with the layers being protected cathodically and the corrosion proceeding laterally rather than towards the substrate.

As shown on the right of FIG. 1, the homogeneous coating 30 of the prior art is disposed to have a single layer covering a substrate. As the sequence shows, over time the hole in the single layer expands in a direction normal to the surface of the substrate until ultimately reaching the substrate, which thereafter is affected by corrosion or other forms of degradation.

In one embodiment, the technology described herein describes a method for producing a multilayer, nanolaminated coating by an electrodeposition process carried out in a single bath, comprising the steps of:

- placing a mandrel or a substrate to be coated in a first electrolyte containing one or more metal ions, ceramic particles, polymer particles, or a combination thereof; and
- applying electric current and varying in time one or more of: the amplitude of the electrical current, electrolyte temperature, electrolyte additive concentration, or electrolyte agitation, in order to produce periodic layers of electrodeposited species or periodic layer of electrodeposited species microstructures; and
- growing a multilayer coating under such conditions until the desired thickness of the multilayer coating is achieved.

Such a method may further comprise after step (c), step (d) removing the mandrel or the substrate from the bath and rinsing.

The technology described herein also sets forth a method for producing a multilayer, nanolaminated coating or cladding using serial electrodeposition in two or more baths comprising the steps of:

- placing a mandrel or substrate to be coated in a first electrolyte containing one or more metal ions, ceramic particles, polymer particles, or a combination thereof; and
- applying electric current and varying in time one or more of: the electrical current, electrolyte temperature, electrolyte additive concentration, or electrolyte agitation, in order to produce periodic layers of electrodeposited species or periodic layer of electrodeposited species microstructures; and

- c) growing a nanometer-thickness layer under such conditions; and
- d) placing said mandrel or substrate to be coated in a second electrolyte containing one or more metal ions that is different from said first electrolyte, said second electrolyte containing metal ions, ceramic particles, polymer particles, or a combination thereof; and
- e) repeating steps (a) through (d) until the desired thickness of the multilayer coating is achieved; wherein steps (a) through (d) are repeated at least two times.

Such a method may further comprise after step (e), step (f) removing the mandrel or the coated substrate from the bath and rinsing.

Corrosion-resistant multilayer coatings can be produced on a mandrel, instead of directly on a substrate to make a free-standing material or cladding. Cladding produced in this manner may be attached to the substrate by other means, including welding, gluing or through the use of other adhesive materials.

The multilayer coatings can comprise layers of metals that are electrolytically deposited from aqueous solution, such as Ni, Zn, Fe, Cu, Au, Ag, Pd, Sn, Mn, Co, Pb and Cr. The multilayer coating can also comprise alloys of these metals, including, but not limited to: ZnFe, ZnCu, ZnCo, NiZn, NiMn, NiFe, NiCo, NiFeCo, CoFe, CoMn. The multilayer can also comprise metals that are electrolytically deposited from a molten salt or ionic liquid solution. These include those metals previously listed, and others, including, but not limited to Al, Mg, Ti and Na. In other embodiments multilayer coatings can comprise one or more metals selected from Ni, Zn, Fe, Cu, Au, Ag, Pd, Sn, Mn, Co, Pb, Al, Ti, Mg and Cr. Alternatively, one or more metals to be electrolytically deposited may be selected from: Ni, Zn, Fe, Cu, Sn, Mn, Co, Pb, Al, Ti, Mg and Cr; or from Ni, Zn, Fe, Cu, Sn, Mn, Co, Ti, Mg and Cr; or from Ni, Zn, Fe, Sn, and Cr.

The multilayer coating can comprise ceramics and polymers that are electrophoretically deposited for aqueous or ionic liquid solutions, including, but not limited to  $\text{Al}_2\text{O}_3$ ,  $\text{SiO}_2$ , TiN,  $\text{Fe}_2\text{O}_3$ ,  $\text{MgO}$ , and  $\text{TiO}_2$ . Suitable polymers include, but are not limited to, epoxy, polyurethane, polyaniline, polyethylene, poly ether ether ketone, polypropylene.

The multilayer coating can also comprise combinations of metals and ceramics, metals and polymers, such as the above-mentioned metals, ceramics and polymers.

The thickness of the individual layers (nanoscale layers) can vary greatly as for example between 0.5 and 10,000 nanometers, and in some embodiments is about 200 nanometers per layer. The thickness of the individual layers (nanoscale layers) may also be about 0.5, 0.7, 1, 2, 5, 10, 15, 20, 25, 30, 40, 50, 75, 100, 200, 400, 500, 1,000, 2,000, 4,000, 6,000, 8,000 or 10,000 nanometers. In other embodiments the layers may be about 0.5 to 1, or 1 to 5, or 5 to 25, or 25 to 100, or 100 to 300, or 100 to 400, or 500 to 1,000, or 1,000 to 2,000, or 2,000 to 5,000, or 4,000 to 10,000 nanometers.

Individual layers may be of the same thickness or different thickness. Layers that vary periodically may also vary in thickness.

The overall thickness of the coating or cladding can vary greatly as, for example, between 2 micron and 6.5 millimeters or more. In some embodiments the overall thickness of the coating or cladding can also be between 2 nanometers and 10,000 nanometers, 4 nanometers and 400 nanometers, 50 nanometers and 500 nanometers, 100 nanometers and 1,000 nanometers, 1 micron to 10 microns, 5 microns to 50 microns, 20 microns to 200 microns, 200 microns to 2

millimeters (mm), 400 microns to 4 mm, 200 microns to 5 mm, 1 mm to 6.5 mm, 5 mm to 12.5 mm, 10 mm to 20 mm, 15 mm to 30 mm.

Layer thickness can be controlled by, among other things, the application of current in the electrodeposition process. This technique involves the application of current to the substrate or mandrel to cause the formation of the coating or cladding on the substrate or mandrel. The current can be applied continuously or, more preferably, according to a predetermined pattern such as a waveform. In particular, the waveform (e.g., sine waves, square waves, sawtooth waves, or triangle waves) can be applied intermittently to promote the electrodeposition process, to intermittently reverse the electrodeposition process, to increase or decrease the rate of deposition, to alter the composition of the material being deposited, or to provide for a combination of such techniques to achieve a specific layer thickness or a specific pattern of differing layers. The current density and the period of the wave forms may be varied independently. In some embodiments current density may be continuously or discretely varied with the range between 0.5 and 2000 mA/cm<sup>2</sup>. Other ranges for current densities are also possible, for example, a current density may be varied within the range between: about 1 and 20 mA/cm<sup>2</sup>; about 5 and 50 mA/cm<sup>2</sup>; about 30 and 70 mA/cm<sup>2</sup>; 0.5 and 500 mA/cm<sup>2</sup>; 100 and 2000 mA/cm<sup>2</sup>; greater than about 500 mA/cm<sup>2</sup>; and about 15 and 40 mA/cm<sup>2</sup> base on the surface area of the substrate or mandrel to be coated. In some embodiments the frequency of the wave forms may be from about 0.01 Hz to about 50 Hz. In other embodiments the frequency can be from: about 0.5 to about 10 Hz; 0.02 to about 1 Hz or from about 2 to 20 Hz; or from about 1 to about 5 Hz.

The multilayer coatings and claddings described herein are suitable for coating or cladding a variety of substrates that are susceptible to corrosion. In one embodiment the substrates are particularly suited for coating substrates made of materials that can corrode such as iron, steel, aluminum, nickel, cobalt, iron, manganese, copper, titanium, alloys thereof, reinforced composites and the like.

The coatings and claddings described herein may be employed to protect against numerous types of corrosion, including, but not limited to corrosion caused by oxidation, reduction, stress (stress corrosion), dissolution, dezincification, acid, base, sulfidation and the like.

#### Example #1

Preparation of a multilayer coating comprising nanoscale layers of zinc-iron alloy, in which the concentration of iron varies in adjacent layers.

A zinc-iron bath is produced using a commercial plating bath formula supplied by MacDermid Inc. (Waterbury, Conn.). The composition of the bath is described in Table 1.

TABLE 1

| Example Plating Bath  |             |           |
|-----------------------|-------------|-----------|
| MacDermid Material    | Composition | Product # |
| Zinc Metal            | 10-12 g/l   | 118326    |
| NaOH                  | 125-135 g/l |           |
| Envirallyo Carrier    | 0.5-0.6%    | 174384    |
| Envirallyo Brightener | 0-0.1%      | 174383    |
| Envirallyo Fe         | 0.2-0.4%    | 174385    |
| Envirallyo C          | 4-6%        | 174386    |
| Envirallyo B          | 0.4-0.6%    | 174399    |

TABLE 1-continued

| Example Plating Bath  |             |           |
|-----------------------|-------------|-----------|
| MacDermid Material    | Composition | Product # |
| Enviralloy Stabilizer | 0.1-0.2%    | 174387    |
| Envirowetter          | 0.05-0.2%   | 174371    |

A steel panel is immersed into the bath and connected to a power supply. The power supply was combined with a computer generated waveform supply that provided a square waveform which alternates between  $25 \text{ mA/cm}^2$  (for 17.14 seconds) and  $15 \text{ mA/cm}^2$  (for 9.52 seconds). The total plating time for a M90 coating (0.9 oz of coating per square foot) is about 1.2 hrs. In this time approximately 325 layers were deposited to achieve a total thickness of 19  $\mu\text{m}$ . The individual layer thickness was between 50 and 100 nm.

The coating is tested in a corrosive environment, in accordance with ASTM B117 (Standard Practice for Operating Salt Spray), and shows no evidence of red rust after 300 hours of exposure.

#### Example #2

Nickel Cobalt alloys have been used extensively in recent history because of its great wear and corrosion resistance. A nanolaminated Ni—Co alloy was created which contains codeposited diamond particles. The Ni—Co alloy by itself is a corrosion and wear resistant alloy. By modulating the electrode potential in the cell, it was possible to laminate the composition of the alloy. By doing this, a galvanic potential difference was established between the layers and thus created a more favorable situation for corrosion and fatigue wear. Also, two unique phases in the crystal structure of the matrix were established. The deposition rate of the diamonds has also been shown to vary with the current density of the cell.

Preparation of a multilayer coating comprising nanoscale layers of a Nickel-Cobalt alloy with diamond codeposition, in which the concentration of the metals vary in adjacent layers.

A traditional Nickel watts bath is used as the basis for the bath. The following table describes all of the components of the bath.

TABLE 2

| Example Plating Bath     |               |
|--------------------------|---------------|
| Component                | Concentration |
| Nickel Sulfate           | 250 g/l       |
| Nickel Chloride          | 30 g/l        |
| Boric Acid               | 40 g/l        |
| Cobalt Chloride          | 10 g/l        |
| SDS                      | .01 g/l       |
| Diamond (<1 micron size) | 5 g/l         |

For creating samples, a steel panel is immersed into the bath and is connected to a power supply. The current density modulation was carried out between  $10 \text{ mA/cm}^2$  and  $35 \text{ mA/cm}^2$  with computer controlled software to form nanoscale layers. The current is applied and varied until a 20  $\mu\text{m}$  thick coating had been formed on the substrate surface.

Testing for this coating has been carried out in a salt fog chamber in accordance with the ASTM B117 standers as well as taber wear tests which show the abrasion resistance

to be significantly better than homogeneous coatings of Nickel-Cobalt and of stainless steel 316.

#### Example #3

Preparation of a Ni—Zr—Cr alloy system containing particulate precursors.

TABLE 3

| Bath Make-up         |             |  |
|----------------------|-------------|--|
| Chemical             | Conc. (g/L) |  |
| Nickel Sulfate       | 312         |  |
| Nickel Chloride      | 45          |  |
| Boric Acid           | 38          |  |
| Surfactant (C-TAB ®) | 0.1         |  |

TABLE 4

| Particle Additions      |             |  |
|-------------------------|-------------|--|
| Particle                | Conc. (g/L) |  |
| Zirconium (1-3 microns) | 40          |  |
| CrC (1-5 microns)       | 15          |  |

#### Bath Make-Up Procedure:

1. Mix metal salts, boric acid and C-Tab at 100° F.
2. Allow full dissolution, then shift pH to between 5 and 6 with ammonium hydroxide
3. Add particles and allow full mixing
4. Particles should be allowed to mix for one day before plating to allow full surfactant coverage

#### Plating Procedure:

1. Substrates should be prepared in accordance with ASTM standards
2. Electrolyte should be held between 100° F. and 120° F.
3. Solution should have sufficient agitation to prevent particle settling, and fluid flow should be even across the substrate
4. A 50% duty cycle pulse waveform at  $75 \text{ mA/cm}^2$  effective current density is applied; the average current density of the pulse waveform can be varied and will vary particle inclusion allowing for a laminated structure with controllable deposit composition.

In a first SEM image of the plated substrates shows a high density particle incorporation of zirconium and chromium carbide particles on a steel substrate. Particle spacing is between  $<1$  and 5 microns and the deposit is fully dense. Particles show relatively even distribution throughout the deposit. A second SEM image shows low particle density inclusions on a steel substrate. Particle spacing is between 1 and 15 microns, with some deposit cleaving at particle/matrix interface. Even particle distribution is less pronounced in the second SEM image. Minor surface roughness is seen in both deposits.

#### Optional Heat Treatment:

In the event the coating requires greater corrosion resistance, a heat treatment can be applied to diffuse included zirconium throughout the deposit, creating, in this case, corrosion-resistant intermetallic phases of the Ni Cr and Zr. Heat treatment may be performed by:

1. Clean the part and dry;
2. Using a furnace of any atmosphere, heat the deposit at no more than 10° C./min up to 927° C.

**11**

3. Hold at 927° C. for 2 hours and  
 4. Air cooling the part.

The above descriptions of exemplary embodiments of methods for forming nanolaminate structures are illustrative of the present invention. Because of variations which will be apparent to those skilled in the art, however, the present invention is not intended to be limited to the particular embodiments described above. The scope of the invention is defined in the following claims.

What is claimed is:

**1. A method comprising:**

forming a coating on a substrate or mandrel, the coating having a thickness from 5 microns to 50 microns and comprising a series of layers arranged in a repeating pattern, each layer of the series of layers having a thickness from about 5 nanometers to about 1,000 nanometers, the series of layers comprising:

A) a first layer of a first alloy that is less noble than the substrate or the mandrel, the first alloy comprising:

i) a first metal in a first concentration that is at least about 1 wt. %, the first metal selected from Co, Fe, Ni, and Zn; and

ii) a second metal in a second concentration that is at least about 1 wt. %; and

B) a second layer of a second alloy that is less noble than the first alloy and less noble than the substrate or the mandrel, the second alloy comprising:

i) the first metal in a third concentration that is at least about 1 wt. %; and

ii) the second metal in a fourth concentration that is at least about 1 wt. %.

2. The method of claim 1, wherein the first metal is Ni or Zn.

3. The method of claim 1, wherein each layer of the series of layers is discrete.

4. The method of claim 1, further comprising a diffuse interface between each layer of the series of layers.

5. The method of claim 1, wherein the second metal is selected from Co, Fe, Ni, and Zn, the second metal being different than the first metal.

6. The method of claim 1, wherein the series of layers further comprises a third layer.

7. The method of claim 1, further comprising forming a cladding by removing the coating from the mandrel.

**8. A method comprising:**

forming a coating on a substrate or mandrel, the coating having a thickness from 5 microns to 50 microns and comprising a series of layers arranged in a repeating pattern, each layer of the series of layers having a thickness from about 5 nanometers to about 1,000 nanometers, the series of layers comprising:

A) a first layer of a first alloy that is more noble than the substrate or the mandrel, the first alloy comprising:

i) Co in a first concentration that is at least about 1 wt. %; and

ii) Ni in a second concentration that is at least about 1 wt. %; and

5

10

20

25

30

35

40

45

50

55

**12**

B) a second layer of a second alloy that is more noble than the first alloy and more noble than the substrate or the mandrel, the second alloy comprising:

i) Co in a third concentration that is at least about 1 wt. %; and

ii) Ni in a fourth concentration that is at least about 1 wt. %; and

C) a third metal layer of a third alloy that is more noble than the substrate or the mandrel, the third alloy comprising:

i) Co in a fifth concentration that is at least about 1 wt. %; and

ii) Ni in a sixth concentration that is at least about 1 wt. %; the first, second, and third alloys being different.

9. The method of claim 8, wherein each layer of the series of layers is discrete.

10. The method of claim 8, further comprising a diffuse interface between each layer of the series of layers.

11. The method of claim 8, further comprising forming a cladding by removing the coating from the mandrel.

**12. A method comprising:**

forming a coating on a substrate or mandrel, the coating having a thickness from 5 microns to 50 microns and comprising a series of layers arranged in a repeating pattern, each layer of the series of layers having a thickness from about 5 nanometers to about 1,000 nanometers, the series of layers comprising:

A) a first layer of a first alloy that is more noble than the substrate or the mandrel, the first alloy comprising:

i) a first metal in a first concentration that is at least about 1 wt. %, the first metal selected from Co, Fe, Ni, and Zn; and

ii) a second metal; and

B) a second layer of a second alloy that is less noble than the first alloy and less noble than the substrate or the mandrel, the second alloy comprising:

i) the first metal in a second concentration that is at least about 1 wt. %; and

ii) the second metal.

13. The method of claim 12, wherein the first metal is Ni or Zn.

14. The method of claim 12, wherein each layer of the series of layers is discrete.

15. The method of claim 12, wherein second metal is selected from Co, Fe, Ni, and Zn, the second metal being different than the first metal.

16. The method of claim 12, wherein the series of layers further comprises a third layer.

17. The method of claim 12, further comprising forming a cladding by removing the coating from the mandrel.

\* \* \* \* \*